



US005391453A

# United States Patent [19]

Ong

[11] Patent Number: 5,391,453  
[45] Date of Patent: Feb. 21, 1995

[54] TONER COMPOSITIONS WITH  
ALUMINUM COMPLEX COMPOSITE  
CHARGE ADDITIVES

[75] Inventor: Beng S. Ong, Mississauga, Canada

[73] Assignee: Xerox Corporation, Stamford, Conn.

[21] Appl. No.: 47,902

[22] Filed: Apr. 19, 1993

[51] Int. Cl.<sup>6</sup> G03G 9/00

[52] U.S. Cl. 430/110; 430/106;  
430/106.6

[58] Field of Search 430/110, 106, 106.6

[56] References Cited

U.S. PATENT DOCUMENTS

4,206,064 6/1980 Kiuchi et al. 430/106

4,298,672 11/1981 Lu ..... 430/108  
4,411,974 10/1983 Lu et al. ..... 430/106  
4,845,003 7/1989 Kiriw et al. ..... 430/110  
5,275,900 1/1994 Ong et al. ..... 430/110

Primary Examiner—Marion E. McCamish

Assistant Examiner—Mark A. Chapman

Attorney, Agent, or Firm—E. O. Palazzo

[57] ABSTRACT

A negatively charged toner composition comprised of resin, colorants comprised of color pigments and/or dyes, optional surface additives, and an aluminum complex composite charge enhancing additive obtained from the reaction of an aqueous aluminum ion solution with a phenol, a hydroxybenzoic acid and a base at a temperature ranging from about 25° C. to about 100° C.

30 Claims, No Drawings

## TONER COMPOSITIONS WITH ALUMINUM COMPLEX COMPOSITE CHARGE ADDITIVES

### BACKGROUND OF THE INVENTION

The invention is generally directed to toner and developer compositions, and more specifically, the present invention is directed to developer and toner compositions containing charge enhancing additives, which impart or assist in imparting a negative charge to toner particles and enable toners with rapid triboelectric charging characteristics. In embodiments, there are provided in accordance with the present invention toner compositions comprised of toner resins, color pigment particles or dye molecules, and certain aluminum complex composites which serve as negative charge enhancing additives. In embodiments, the present invention is directed to toner compositions with aluminum complex composite charge enhancing additives, which additives can be obtained from the reaction of aluminum ion with a phenol and a hydroxybenzoic acid under basic reaction conditions at a temperature ranging from ambient, about 25° C. to about 100° C. The aluminum complex composite charge enhancing additives in embodiments are believed to be comprised of or contain active aluminum complex components of tetra-coordinated and/or hexa-coordinated aluminum complex anions with mixed ligands derived from hydroxybenzoic acid and phenol, and counter cations of a proton, an alkaline metal ion, or an ammonium ion. The aluminum complex composite charge enhancing additives in embodiments of the present invention enable, for example, toners with rapid triboelectric charging characteristics, extended developer life, stable triboelectrical properties irrespective of changes in environmental conditions, and high image print quality with substantially no background deposits. Also, the aforementioned toner compositions usually contain a colorant component comprised of, for example, carbon black, magnetites, or mixtures thereof, color pigments or dyes of cyan, magenta, yellow, blue, green, red, or brown color, or mixtures thereof thereby providing for the development and generation of black only and colored images. The toner and developer compositions of the present invention can be selected for electrophotographic, especially xerographic, imaging and printing processes, including color processes.

Toners with negative charge additives are known, reference for example U.S. Pat. Nos. 4,411,974 and 4,206,064, the disclosures of which are totally incorporated herein by reference. The '974 patent discloses negatively charged toner compositions comprised of toner resins, color pigments, and as a charge enhancing additive ortho-halophenyl carboxylic acids. Similarly, there are disclosed in the '064 patent toner compositions with chromium, cobalt, and nickel complexes of salicylic acid as negative charge enhancing additives. In U.S. Pat. No. 4,845,003, there are illustrated negatively charged toners with certain aluminum salt charge additives. More specifically, this patent discloses as charge additives aluminum complexes comprised of two or three hydroxybenzoic acid ligands bonded to a central aluminum ion. While these charge additives may have the capability of imparting negative triboelectric charge to toner particles, they are generally not efficient in promoting the rate of triboelectric charging of toner particles. A fast rate of triboelectric charging is particularly crucial for high speed xerographic machines since,

for example, these machines consume toner rapidly, and fresh toner has to be constantly added. The added uncharged toners, therefore, must charge up to their equilibrium triboelectric charge level rapidly to ensure no interruption in the xerographic imaging or printing operation. Another disadvantage of these charge additives is their thermal instability, that is they often break down during the thermal extrusion process of the toner manufacturing cycle. Most or many of these and other disadvantages are eliminated, or substantially eliminated with the metal complex charge additives of the present invention.

Developer compositions with charge enhancing additives, which impart a positive charge to the toner particles, are also well known. Thus, for example, there is described in U.S. Pat. No. 3,893,935 the use of quaternary ammonium salts as charge control agents for electrostatic toner compositions; U.S. Pat. No. 4,221,856, which discloses electrophotographic toners containing resin compatible quaternary ammonium compounds in which at least two R radicals are hydrocarbons having from 8 to about 22 carbon atoms, and each other R is a hydrogen or hydrocarbon radical with from 1 to about 8 carbon atoms, and A is an anion, for example, sulfate, sulfonate, nitrate, borate, chlorate, and the halogens such as iodide, chloride and bromide, reference the Abstract of the Disclosure and column 3; a similar teaching is presented in U.S. Pat. No. 4,312,933 which is a division of U.S. Patent 4,291,111; similar teachings are presented in U.S. Pat. No. 4,291,112 wherein A is an anion including, for example, sulfate, sulfonate, nitrate, borate, chlorate, and the halogens; U.S. Pat. No. 4,338,390, the disclosure of which is totally incorporated herein by reference, discloses developer compositions containing as charge enhancing additives organic sulfate and sulfonates, which additives can impart a positive charge to the toner composition; and U.S. Pat. No. 4,298,672, the disclosure of which is totally incorporated herein by reference, discloses positively charged toner compositions with resins and pigment particles, and as charge enhancing additives alkyl pyridinium compounds.

Illustrated in U.S. Pat. No. 5,275,900 is a negatively charged toner composition comprised of a polymer or polymer resins, a colorant or colorants, optional surface additives, and a metal complex charge enhancing additive obtained from the reaction of a hydroxybenzoic acid and a base with a mixture of a metal ion and a hydroxyphenol; U.S. Pat. No. 5,300,387, which discloses a negatively charged toner composition comprised of a polymer or polymers, a colorant or colorants, optional surface additives, and a metal complex charge enhancing additive obtained from the reaction of a hydroxybenzoic acid and a base with a mixture of a metal ion and an aromatic dicarboxylic acid; U.S. Pat. No. 5,238,768, which discloses a negatively charged toner composition comprised of resin particles, colorants, optional surface additives, and a dihydroxyaryl sulfone charge enhancing additive, or an unsymmetrical hydroxyaryl sulfone charge enhancing additive obtained from the condensation of sulfuric acid with a molar equivalent of a phenol, followed by condensation with a second phenol, or from the condensation of an aromatic sulfonic acid with a phenol; U.S. Ser. No. 964,544 (D/92402), which discloses a toner composition comprised of polymers, pigment particles and/or dyes, optional surface additives, and a charge enhancing addi-

tive derived from the reaction of a metal, a metal carbonyl, a metal salt, or a metal oxide, with a  $\beta$ -diketone, a  $\beta$ -keto ester, or a malonic ester in an aqueous medium or organic medium; U.S. Pat. No. 5,238,768, which discloses a negatively charged toner composition comprised of a polymer resin or polymer resins, colorants comprised of pigment particles and/or dyes, optional surface additives, and a nonionic zinc complex charge enhancing additive containing two different ligands derived from an ortho-hydroxyphenol and an ortho-hydroxybenzoic acid; U.S. Pat. No. 5,256,575, which discloses a negatively charged toner composition comprised of resin particles, pigment particles, optional surface additives, and a halogenated salicylic acid complex charge enhancing additive of the following formula



wherein Z is zinc or chromium; M is hydrogen, an alkali metal, an alkaline earth metal,  $\text{NH}_4$ , or  $\text{NR}_4$  wherein R is alkyl; X and Y are independently selected from the group consisting of chloride, iodide and bromide; and n and m are the numbers 1 or 2; U.S. Pat. No. 5,256,514, which discloses a negatively charged toner composition comprised of resin particles, pigment particles, optional surface additives, and a halogenated salicylic acid charge enhancing additive of the following formula



wherein X is halogen; M is hydrogen, an alkaline earth, an alkali metal, or  $\text{NR}_4$  wherein R is alkyl; and n is the number 1 or 2; and U.S. Pat. No. 5,300,389, which discloses a negatively charged toner composition comprised of resin particles, pigment particles, optional surface additives, and a halogenated aluminum salicylic acid complex charge enhancing additive of the following formulas



or

-continued



wherein M is hydrogen, an alkali metal, an alkaline earth metal,  $\text{NH}_4$ , or  $\text{NR}_4$  wherein R is alkyl; X and Y are independently selected from the group consisting of iodide, chloride and bromide, and n and m are the numbers 1 or 2, the disclosures of which are totally incorporated herein by reference.

Known aluminum complexes, such as bis(3,5-di-tert-butylsalicylato)aluminum or bis(4-tert-butylcatecholato)aluminum complexes, may not in many instances be considered acceptable negative charge control agents since, for example, the former has a slow admix time, while the latter generally imparts unacceptably low negative tribo to toners. For example, when used as surface CCA (at 0.1 to 0.25 weight percent level) on a toner comprised of styrene butadiene resin and 6 weight percent of REGAL 330® carbon black, potassium bis(3,5-di-tert-butylsalicylato)aluminum (III) imparted a negative tribo to the toner of -15 to -40 microcoulombs/gram with polyvinylidene steel coated carrier, however, it could not meaningfully improve the toner's admix time of 2 to 5 minutes. Potassium bis(4-tert-butylcatecholato)aluminum (III) enhanced the toner's admix performance (>15 seconds), but it failed to impart a useful magnitude of negative tribo to the toner (<10 microcoulombs/gram).

While many charge enhancing additives are known, there continues to be a need for charge enhancing additives, which when incorporated in toners provide many of the advantages illustrated herein. There is also a need for negative charge enhancing additives which are useful for incorporation into black and colored toner compositions which can be utilized for developing positive electrostatic latent images. Moreover, there is a need for colored toner compositions containing charge enhancing additives which do not interfere with the color quality of the colorants present in the toners. Another need relates to the provision of toner compositions with certain charge enhancing additives, which toners in embodiments thereof possess substantially stable triboelectric charge levels, and display acceptable rates of triboelectric charging characteristics. Furthermore, there is also a need for toner compositions with charge enhancing additives which possess excellent dispersibility characteristics in toner resins, and can, therefore, form stable dispersions in toner compositions. There is also a need for negatively charged black and colored toner compositions that are useful for incorporation into various imaging processes, inclusive of color xerography, as illustrated in U.S. Pat. No. 4,078,929, the disclosure of which is totally incorporated herein by reference; laser printers; and additionally a need for toner compositions useful in imaging apparatuses having incorporated therein layered photoresponsive imaging members, such as the members illustrated in U.S. Pat. No. 4,265,990, the disclosure of which is totally incor-

porated herein by reference. Also, there is a need for negative toner compositions which have desirable triboelectric charge levels of, for example, from between about -10 to about -40 microcoulombs per gram, and triboelectric charging rates of less about 120 seconds, and preferably less than 60 seconds as measured by standard charge spectrograph methods when the toners are frictionally charged against suitable carrier particles via roll milling. There is also a need for nontoxic, substantially nontoxic, or environmentally compatible charge enhancing additives which when incorporated at effective concentrations of, for example, less than 10 weight percent, and preferably less than 5 weight percent in toners, such as 0.1 to about 3 weight percent, render the toners to be environmentally acceptable. An additional need resides in the provision of simple and cost-effective preparative processes for the aluminum complex composite charge enhancing additives of the present invention. The concentrations of the charge enhancing additives that may be incorporated into the toner compositions generally range from about 0.05 weight percent to about 5 weight percent, depending on whether the charge additive is utilized as a surface additive or as a dispersion in the bulk of the toner. The effective concentrations of toner in the developer, that is toner and carrier particles, are, for example, from about 0.5 to about 5 weight percent, and preferably from about 1 to about 3 weight percent.

#### SUMMARY OF THE INVENTION

It is an object of the present invention to provide toner and developer compositions with negative charge enhancing additives.

In another object of the present invention there are provided negatively charged toner compositions useful for the development of electrostatic latent images.

In yet a further object of the present invention there may be provided, it is believed, humidity insensitive, from about, for example, 20 to 80 percent relative humidity at temperatures of from 60° to 80° F. as determined in a relative humidity testing chamber, negatively charged toner compositions with desirable triboelectric charging rates of less than 120 seconds, and preferably less than 60 seconds as determined by the charge spectrograph method when toner particles are frictionally charged against suitable carrier particles via roll milling, and acceptable triboelectric charging levels of from about -10 to about -40 microcoulombs per gram.

Another object of the present invention resides in the preparation of negative toners which will enable the development of images in electrophotographic imaging apparatuses, which images have substantially no background deposits thereon, are substantially smudge proof or smudge resistant and, therefore, are of excellent resolution; and further, such toner compositions can be selected for high speed electrophotographic apparatuses, that is for example those exceeding 50 copies per minute.

A further object is to provide a simple and cost-effective preparative processes for the aluminum complex composite charge enhancing additives of the present invention, and which complexes can in embodiments be considered mixed ligands of phenols and o-hydroxybenzoic acids obtained by reacting aluminum sulfate with potassium-o-hydroxy benzoate in the presence of an excess of phenol under basic conditions.

These and other objects of the present invention may be accomplished in embodiments thereof by providing toner compositions comprised of toner resins, colorants comprised of color pigments or dyes, and certain aluminum complex composite charge enhancing additives prepared by reacting an aluminum ion with a phenol and a hydroxybenzoic acid in the presence of a base, such as for example an alkaline component like sodium hydroxide, potassium hydroxide, an amine, and the like. More specifically, the present invention in embodiments is directed to toner compositions comprised of toner resins, pigment particles, and an aluminum complex composite additive containing active components as essentially represented by Formulas (I), (II), or mixtures thereof in embodiments



wherein R is a substituent such as hydrogen, halide like chloride, bromide, iodide, alkyl with, for example, 1 to about 25 carbon atoms, aryl with, for example, 6 to about 24 carbon atoms, alkoxy with, for example, 1 to about 25 carbon atoms, aryloxy with, for example, 6 to about 24 carbon atoms, hydroxy, nitro, amino, and the like; Ar represents an aromatic group such as phenyl, tolyl, xylyl, anisyl, nitrophenyl, and the like; M+ is a proton, an alkaline metal cation, or an ammonium ion; and m is a number of from 1 to about 3.

Examples of alkyl and alkoxy preferably include those with 1 to about 10 carbon atoms, such as methyl, methoxy, ethyl, ethoxy, propyl, propoxy, butyl, butoxy, pentyl, pentoxy, hexyl, hexoxy, heptyl, heptoxy, octyl, octoxy, and the like. Aryl includes those with from 6 to about 24 carbon atoms such as phenyl, xylyl, anisyl and the like as illustrated herein. Examples of counter cation M+ are K+, Na+, Cs+, NH4+, RNH3+, R2NH2+, R3NH+, R4N+, wherein R is as illustrated herein and is preferably alkyl of 1 to about 10 carbon atoms, and the like. Aryloxy includes known substituents such as phenoxy, methylphenoxy, chlorophenoxy, and the like. Halide includes chloride, bromide, iodide, and fluoride.

The aforementioned charge additives can be incorporated into the toner, may be present on the toner surface, or may be present on toner surface additives such as colloidal silica particles. Various effective amounts of charge additive can be selected, such as for example from about 0.05 to about 10, and preferably from about 1 to about 3 weight percent in embodiments. Advantages of rapid triboelectric charging characteristics of generally less than 120 seconds, and preferably less than 60 seconds in embodiments as measured by the standard charge spectrograph methods when the toners are frictionally charged against carrier particles by roll mixing

methods, appropriate triboelectric charge levels, and the like can be achieved with many of the aforementioned toners of the present invention. In another embodiment of the present invention, there are provided, subsequent to known micronization and classification, toner particles with a volume average diameter of from about 5 to about 20 microns.

Illustrative specific examples of the active aluminum complex component (I) of the present invention include potassium (3,5-di-t-butylsalicylato)-bis(4-t-butylphenolato)aluminum (III); (3,5-di-t-butylsalicylato)-bis(phenolato)aluminum (III); (3,5-di-iodosalicylato)-bis(4-t-butylphenolato)aluminum (III); (3,5-di-iodosalicylato)-bis(phenolato)aluminum (III); (3,5-di-iodosalicylato)-bis(4-iodophenolato)aluminum (III); (3,5-di-iodosalicylato)-bis(3-iodophenolato)aluminum (III); (3,5-di-t-butyl-salicylato)-bis(4-iodophenolato)aluminum (III); (5-iodosalicylato)-bis(3-iodophenolato)aluminum (III); (3,5-di-t-butylsalicylato)-bis(4-methoxyphenolato)aluminum (III); (3,5-di-iodosalicylato)-bis(3-methoxyphenolato)aluminum (III); and (3,5-di-t-butylsalicylato)-bis(4-methylphenolato)aluminum (III); while illustrative examples of the active aluminum complex component (II) of the present invention include bis(4-t-butylphenolato)-bis(3,5-di-t-butylsalicylato)aluminum (III), bis(phenolato)-bis(3,5-di-t-butylsalicylato)aluminum (III); bis(4-t-butylphenolato)-bis(3,5-di-iodosalicylato)aluminum (III); bis(phenolato)-bis(3,5-di-iodosalicylato)aluminum (III); bis(4-iodophenolato)-bis(3,5-di-t-butylsalicylato)aluminum (III); bis(3-iodophenolato)-bis(3,5-di-iodosalicylato)aluminum (III); bis(4-iodophenolato)-bis(3,5-di-t-butylsalicylato)aluminum (III); bis(3-iodophenolato)-bis(5-iodosalicylato)aluminum (III); bis(4-methoxyphenolato)-bis(3,5-di-t-butylsalicylato)aluminum (III); bis(3-methoxyphenolato)-bis(3,5-di-iodosalicylato)aluminum (III); and bis(4-methylphenolato)-bis(3,5-di-t-butylsalicylato)aluminum (III).

The aluminum complex composite charge additives of the present invention can be prepared by treating an aqueous aluminum ion solution with a phenol and a base, and then with a hydroxybenzoic acid. During the reaction, the pH of the reaction mixture is maintained at above 7 by addition of a base. The reaction is generally accomplished at an effective temperature of, for example, between ambient and the refluxing temperature of the reaction mixture for a duration ranging from 20 minutes to about 10 hours. Alternatively, the composite charge enhancing additives can also be obtained by treating an aqueous aluminum ion solution containing a phenol with an aqueous solution of hydroxybenzoic acid and a base at a pH above 7 and a reaction temperature of from ambient to the refluxing temperature of the reaction medium. After the reaction, the resulting aluminum complex composite product is filtered and washed with water or dilute aqueous base. In embodiments of the present invention, the aluminum complex composite additives obtained may contain a mixture of proton and alkaline metal cation or ammonium ion as the counter cations. In another specific embodiment, the present invention is directed to aluminum complex composite charge additives derived from the reaction of aluminum ion with an ortho-hydroxybenzoic acid (salicylic acid) and a phenol.

The toner compositions of the present invention can be prepared by a number of known methods such as admixing and heating toner resins such as styrene buta-

diene copolymers, colorants such as color pigment particles or dye compounds, and the aforementioned aluminum complex composite charge enhancing additives in a concentration preferably ranging from about 0.5 percent to about 5 percent, in a toner extrusion device, such as the ZSK53 available from Werner Pfleiderer, and removing the resulting toner composition from the device. Subsequent to cooling, the toner composition is subjected to grinding utilizing, for example, a Sturtevant micronizer for the purpose of achieving toner particles with a volume average diameter of preferably from about 3 to about 15 microns, which diameters are determined by a Coulter Counter. Subsequently, the toner compositions can be classified utilizing, for example, a Donaldson Model B classifier for the purpose of removing unwanted fine toner particles.

Illustrative examples of suitable toner resins selected for the toner and developer compositions of the present invention include vinyl polymers such as styrene polymers, acrylonitrile polymers, vinyl ether polymers, acrylate and methacrylate polymers; epoxy polymers; polyurethanes; polyamides and polyimides; polyesters; and the like. The polymer resins selected for the toner compositions of the present invention include homopolymers or copolymers of two or more monomers. Furthermore, the above mentioned polymer resins may also be crosslinked depending on the desired toner properties. Illustrative vinyl monomer units in the vinyl polymers include styrene, substituted styrenes, chlorostyrene, methyl acrylate and methacrylate, ethyl acrylate and methacrylate, propyl acrylate and methacrylate, butyl acrylate and methacrylate, pentyl acrylate and methacrylate, butadiene, vinyl chloride, acrylonitrile, acrylamide, alkyl vinyl ether and the like. Illustrative examples of the dicarboxylic acid units in the polyester resins suitable for use in the toner compositions of the present invention include phthalic acid, terephthalic acid, isophthalic acid, succinic acid, glutaric acid, adipic acid, pimelic acid, suberic acid, azelaic acid, sebacic acid, maleic acid, fumaric acid, dimethyl glutaric acid, bromoadipic acid, dichloroglutaric acid, and the like; while illustrative examples of the diol units in the polyester resins include ethanediol, propanediols, butanediols, pentanediols, pinacol, cyclopentanediols, hydrobenzoin, bis(hydroxyphenyl)alkanes, dihydroxybiphenyl, substituted dihydroxybiphenyls, and the like.

As one toner resin, there are selected polyester resins as illustrated in U.S. Pat. No. 3,590,000, the disclosure of which is totally incorporated herein by reference; polyester resins obtained from the reaction of bisphenol A and propylene oxide, followed by the reaction of the resulting product with fumaric acid, and branched polyester resins resulting from the reaction of dimethylterephthalate with 1,3-butanediol, 1,2-propanediol, and pentanetriol. Further, low melting polyesters, especially those prepared by reactive extrusion, reference U.S. Ser. No. 814,641 (D/91117), and U.S. Pat. No. 5,227,460, the disclosures of which are totally incorporated herein by reference, can be selected as toner resins. Other specific toner resins include styrene-methacrylate copolymers, and styrene-butadiene copolymers; PLIOLITES®; suspension polymerized styrene-butadienes, reference U.S. Pat. No. 4,558,108, the disclosure of which is totally incorporated herein by reference. Also, waxes with a molecular weight of from about 1,000 to about 6,000, such as polyethylene, poly-

propylene, and paraffin waxes, can be included in, or on the toner compositions as fuser roll release agents.

The toner resins are present in a sufficient, but effective amount, for example from about 30 to about 95 weight percent. Thus, when 1 percent by weight of the charge enhancing additive is present, and 10 percent by weight of colorant, such as carbon black or color pigment, is contained therein, about 89 percent by weight of resin is selected. Also, the composite charge enhancing additive of the present invention may be applied as a surface coating on the toner particles. When used as a coating, the charge enhancing additive of the present invention is present in an amount of from about 0.05 weight percent to about 5 weight percent, and preferably from about 0.1 weight percent to about 1.0 weight percent.

Numerous well known suitable color pigments or dyes can be selected as the colorant for the toner compositions including, for example, carbon black like REGAL 330®, nigrosine dye, metal phthalocyanines, aniline blue, magnetite, or mixtures thereof. The colorant, which is preferably carbon black or other color pigments, should be present in a sufficient amount to render the toner composition with a sufficiently high color intensity. Generally, the colorants are present in amounts of from about 1 weight percent to about 20 weight percent, and preferably from about 2 to about 10 weight percent based on the total weight of the toner composition; however, lesser or greater amounts of colorant can be selected.

When the pigments are comprised of magnetites or a mixture of magnetites and color pigment particles, thereby enabling single component toners and toners for magnetic ink character recognition (MICR) applications in some instances, which magnetites are a mixture of iron oxides ( $FeO.Fe_2O_3$ ), including those commercially available as MAPICO BLACK®, they are present in the toner composition in an amount of from about 5 weight percent to about 60 weight percent, and preferably in an amount of from about 10 weight percent to about 50 weight percent. Mixtures of carbon black and magnetite with from about 1 to about 15 weight percent of carbon black, and preferably from about 2 to about 6 weight percent of carbon black, and magnetite, such as MAPICO BLACK®, in an amount of, for example, from about 5 to about 60, and preferably from about 10 to about 50 weight percent can be selected for black toner compositions of the present invention.

There can also be blended with the toner compositions of the present invention external additives including flow aid additives, which additives are usually present on the surface thereof. Examples of these additives include colloidal silicas such as AEROSIL®, metal salts and metal salts of fatty acids inclusive of zinc stearate, aluminum oxides, cerium oxides, titanium oxides, and mixtures thereof, which additives are generally present in an amount of from about 0.1 percent by weight to about 5 percent by weight, and preferably in an amount of from about 0.5 percent by weight to about 2 percent by weight. Several of the aforementioned additives are illustrated in U.S. Pat. Nos. 3,590,000 and 3,800,588, the disclosures of which are totally incorporated herein by reference.

With further respect to the present invention, colloidal silicas, such as AEROSIL®, can be surface treated with the aluminum complex composite charge additives of the present invention illustrated herein in an amount of from about 1 to about 50 weight percent and prefera-

bly 10 weight percent to about 25 weight percent followed by the addition thereof to the toners in an amount of from 0.1 to 10 and preferably 0.1 to 5 weight percent.

Also, there can be included in the toner compositions of the present invention low molecular weight waxes, such as polypropylenes and polyethylenes commercially available from Allied Chemical and Petrolite Corporation, EPOLENE N-15™ commercially available from Eastman Chemical Products, Inc., VISCOL 550-P™, a low weight average molecular weight polypropylene available from Sanyo Kasei K.K., and similar materials. The commercially available polyethylenes selected have a molecular weight of from about 1,000 to about 1,500, while the commercially available polypropylenes utilized for the toner compositions of the present invention are believed to have a molecular weight of from about 4,000 to about 5,000. Many of the polyethylene and polypropylene compositions useful in the present invention are illustrated in British Patent No. 1,442,835, the disclosure of which is totally incorporated herein by reference. These low molecular weight wax materials are present in the toner composition of the present invention in various amounts, however, generally these waxes are present in the toner composition in an amount of from about 1 percent by weight to about 15 percent by weight, and preferably in an amount of from about 2 weight percent to about 10 weight percent.

Encompassed within the scope of the present invention are colored toner and developer compositions comprised of toner resins, optional carrier particles, the charge enhancing additives illustrated herein, and as colorants red, blue, green, brown, magenta, cyan and/or yellow dyes or color pigments, as well as mixtures thereof. More specifically, with regard to the generation of color images utilizing a developer composition with the charge enhancing additives of the present invention, illustrative examples of magenta materials that may be selected as colorants include, for example, 2,9-dimethyl-substituted quinacridone and anthraquinone dye identified in the Color Index as CI 60710, CI Dispersed Red 15, diazo dye identified in the Color Index as CI 26050, CI Solvent Red 19, and the like. Illustrative examples of cyan materials that may be used as colorants include copper phthalocyanine, x-copper phthalocyanine pigment listed in the Color Index as CI 74160, CI Pigment Blue, and Anthrathrene Blue, identified in the Color Index as CI 69810, Special Blue X-2137, and the like; while illustrative examples of yellow pigments that may be selected are diarylide yellow 3,3-dichlorobenzidene acetoacetanilides, a monoazo pigment identified in the Color Index as CI 12700, CI Solvent Yellow 16, a nitrophenyl amine sulfonamide identified in the Color Index as Foron Yellow SE/GLN, CI Dispersed Yellow 33, 2,5-dimethoxy-4-sulfonanilide phenylazo-4'-chloro-2,5-dimethoxy acetoacetanilide, and Permanent Yellow FGL. The aforementioned colorants are incorporated into the toner composition in various suitable effective amounts providing the objectives of the present invention are achieved. In one embodiment, these colorants are present in the toner composition in an amount of from about 1 percent by weight to about 15 percent by weight based on the total weight of the toner.

For the formulation of developer compositions, there are mixed with the toner particles carrier components, particularly those that are capable of triboelectrically assuming an opposite polarity to that of the toner com-

position. Accordingly, the carrier particles of the present invention are selected to be those that would render the toner particles negatively charged while acquiring a positive charge polarity themselves via frictional charging against the toner particles of the present invention. The opposite charge polarities of the carrier and toner particles of the developer composition thus ensure the toner particles to adhere to and surround the carrier particles. Illustrative examples of carrier particles include iron powder, steel, nickel, iron, ferrites, including copper zinc ferrites, nickel zinc ferrites, and the like. Additionally, there can be selected as carrier particles nickel berry carriers as illustrated in U.S. Pat. No. 3,847,604, the disclosure of which is totally incorporated herein by reference. The selected carrier particles can be used with or without a coating, the coating generally containing terpolymers of styrene, methylmethacrylate, and a silane, such as triethoxysilane, reference U.S. Pat. Nos. 3,526,533 and 3,467,634, the disclosures of which are totally incorporated herein by reference; polymethylmethacrylates; other known coatings; and the like. The carrier particles may also include in the coating, which coating can be present in one embodiment in an amount of from about 0.1 to about 3 weight percent, conductive substances such as carbon black in 25 an amount of from about 5 to about 30 percent by weight. Polymer coatings not in close proximity in the triboelectric series can also be selected, reference U.S. Pat. Nos. 4,937,166 and 4,935,326, the disclosures of which are totally incorporated herein by reference, including for example KYNAR® and polymethylmethacrylate mixtures (40/60). Coating weights can vary as indicated herein; generally, however, from about 0.3 to about 2, and preferably from about 0.5 to about 1.5 weight percent coating weight is selected. 30

Furthermore, the diameter of the carrier particles, preferably spherical in shape, is generally from about 50 to about 1,000 microns, and preferably from between about 80 and 200 microns in volume average diameter thereby permitting them, for example, to possess sufficient density and inertia to avoid adherence to the electrostatic images during the development process. The carrier component can be mixed with the toner composition in various suitable combinations, such as about 1 to 5 parts by weight of toner to 100 parts by weight of 45 carrier particles.

The toner composition of the present invention can be prepared by a number of known methods including extrusion melt blending the toner resins, colorants, and the aluminum complex charge enhancing additive of the present invention as indicated herein, followed by mechanical attrition and classification. Other methods include those well known in the art such as spray drying, melt dispersion, extrusion processing, dispersion polymerization, and suspension polymerization. Also, as indicated herein the toner composition without the charge enhancing additive can be first prepared, followed by addition of the charge enhancing additives and other optional surface additives, or the charge enhancing additive-treated surface additives such as colloidal silicas. Further, other methods of preparation for the toner are as illustrated herein.

The toners of the present invention are usually jetted and classified subsequent to preparation to enable toner particles with a preferred volume average diameter of from about 3 to about 15 microns. The triboelectric charging rates for the toners of the present invention are preferably less than 120 seconds, and more specifically,

less than 60 seconds in embodiments thereof as determined by the known charge spectrograph method as described hereinbefore. These toner compositions with rapid rates of triboelectric charging characteristics enable, for example, the development of images in electrophotographic imaging apparatuses, which images have substantially no background deposits thereon, even at high toner dispensing rates in some instances, for instance exceeding 20 grams per minute; and further, such toner compositions can be selected for high speed electrophotographic apparatuses, that is those exceeding 50 copies per minute.

The toner and developer compositions of the present invention may be selected for use in electrostatographic imaging apparatuses containing therein conventional photoreceptors providing that they are capable of forming positive electrostatic latent images relative to the triboelectric charge polarity of the toners.

The following Examples are being supplied to further illustrate various embodiments of the present invention, it being noted that these Examples are intended to illustrate and not limit the scope of the present invention. Comparative Examples are also presented.

#### EXAMPLE I

An aluminum complex composite additive derived from aluminum sulfate, 3,5-di-tert-butylsalicylic acid and 4-tert-butylphenol was prepared as follows:

An aqueous solution of 16.70 grams of aluminum sulfate octadecahydrate in 100 milliliters of water was mechanically stirred and heated to 90° C. in a 500 milliliter round-bottomed flask fitted with a water condenser. An aqueous solution of 15.0 grams of 4-tert-butylphenol and 6.60 grams of 85 percent potassium hydroxide in 30 milliliters of water was added dropwise over a period of about 15 minutes. After 30 minutes of reaction, the pH of the reaction mixture was adjusted from 4 to 8 by adding aqueous potassium hydroxide solution. The mixture was then allowed to react for another 1 hour before addition of 12.5 grams of 3,5-di-tert-butylsalicylic acid. After 1 hour of reaction, the pH of the reaction mixture was again adjusted to 8 with aqueous potassium hydroxide solution. Subsequently, the mixture was stirred at 90° C. for another hour before cooling down to room temperature and filtered. The filtered cake was washed with dilute aqueous potassium hydroxide solution, and dried in vacuo at 80° C. for 48 hours. The yield of the aluminum complex composite product was 24.1 grams.

#### EXAMPLE II

An aluminum complex composite additive derived from aluminum sulfate, 3,5-di-tert-butylsalicylic acid and 4-tert-butylphenol was also prepared by the following procedure:

A mixture of 8.50 grams of aluminum sulfate octadecahydrate, 8.45 grams of 4-tert-butylphenol and 150 milliliters of water were mechanically stirred and heated to 90° C. in a 1 liter round-bottomed flask fitted with a water condenser. An aqueous solution of 12.52 grams of 3,5-di-tert-butylsalicylic acid and 6.60 grams of 85 percent potassium hydroxide in 150 milliliters of water was added dropwise at a rate of about 10 milliliters/minute. The resulting mixture was stirred for 3 hours, and then cooled down to about 60° C. After adjusting its pH to about 7, the reaction mixture was filtered, and the filtered cake was washed with dilute aqueous potassium solution. The yield of the aluminum complex composite

product, after drying in vacuo at 80° C. for 48 hours, was 14.4 grams.

### EXAMPLE III

An aluminum complex composite additive derived from aluminum sulfate, 3,5-di-iodosalicylic acid and 4-tert-butylphenol was prepared according to the procedure of Example I with the exception that 19.50 grams of 3,5-di-iodosalicylic acid was utilized in place of 12.5 grams of 3,5-di-tert-butylsalicylic acid. The yield of the aluminum complex composite product was 28.2 grams.

### EXAMPLE IV

There was prepared in an extrusion device, available as ZSK-30 from Werner Pfleiderer, a toner composition by adding thereto 94.0 weight percent of a suspension polymerized styrene butadiene resin, reference U.S. Pat. No. 4,558,108, the disclosure of which is totally incorporated herein by reference, and 6.0 weight percent of REGAL 330® carbon black. The toner composition was extruded at a rate of 20 pounds per hour at a temperature of about 130° C. with a screw speed of 200 rpm. The strands of melt mixed product exiting from the extruder were air cooled, pelletized in a Berlyn Pelletizer and then fitzmilled in a Model J Fitzmill. The toner product was then subjected to grinding in a Sturtevant micronizer. Thereafter, the aforementioned toner particles were classified in a Donaldson Model B classifier for the purpose of removing fine particles, that is those with a volume average diameter of less than 4 microns. The resulting toner had a volume average particle diameter of 10.6 microns, and a particle size distribution of 1.22 as measured by a Coulter Counter. Subsequently, the toner was surface coated with 0.25 weight percent of the aluminum complex composite charge enhancing additive of Example I by roll-milling for 30 to 60 seconds.

The above treated toner was equilibrated at room temperature under 50 percent relative humidity for 24 hours. A developer was then prepared by blending 2.0 weight percent of the prepared surface treated toner with 98.0 weight percent of a carrier containing a nickel zinc ferrite core and 0.9 weight percent of a polymer composite coating comprised of 80 weight percent of a methyl terpolymer and 20 weight percent of Vulcan XC72R carbon black. The methyl terpolymer was comprised of about 81 weight percent of polymethyl methacrylate and 19 weight percent of a styrene vinyltriethoxysilane polymer. The developer was roll milled for 30 minutes to generate the time zero developer, and the triboelectric charge of the toner was measured to be -28.4 microcoulombs per gram by the standard blow-off technique in a Faraday Cage apparatus. To measure the rate of triboelectric charging of toner, 1.0 weight percent of the above prepared uncharged toner was added to the above time zero developer, and the charge distribution of the toner of the resulting developer was measured as a function of the roll milling time using a charge spectrograph. The time required for the toner of the resulting developer to attain a charge distribution similar to that of the toner of the time zero developer was taken to be the rate of charging of the toner. For the uncharged toner, the rate of charging was about 30 seconds.

### COMPARATIVE EXAMPLE 1

A comparative black toner with the charge enhancing additive, BONTRON E-88® tris(3,5-di-t-butyl salicylato)aluminum, it is believed, obtained from Orient Chemicals, reference U.S. Pat. No. 4,845,003, the disclosure of which is totally incorporated herein by reference, was prepared by blending the untreated toner of Example IV with 0.25 weight percent of BONTRON E-88®, and a developer was then prepared from this toner in accordance with the procedure of Example IV. The toner exhibited a triboelectric charge of -40.4 microcoulombs per gram, and its rate of charging was measured to be about 5 minutes.

### EXAMPLE V

A black toner was prepared in accordance with the procedure of Example IV using 0.25 weight percent of the aluminum complex composite charge enhancing additive of Example II instead of Example I. A developer was then prepared from this toner in accordance with the procedure of Example IV. The prepared toner had a triboelectric charge of -25.5 microcoulombs per gram, and a rate of charging of about 30 seconds.

### EXAMPLE VI

A black toner was prepared in accordance with the procedure of Example IV with 0.25 weight percent of the aluminum complex composite charge enhancing additive of Example III instead of Example I. A developer was then prepared from this toner in accordance with the procedure of Example IV. The prepared toner displayed a triboelectric charge of -31.1 microcoulombs per gram, and its rate of charging was measured to be about 30 seconds.

### COMPARATIVE EXAMPLE 2

A comparative black toner with 0.25 weight percent of the charge enhancing additive, BONTRON E-84® obtained from Orient Chemicals, reference U.S. Pat. No. 4,845,003, the disclosure of which is totally incorporated herein by reference, was prepared by blending the untreated toner of Example IV with 0.25 weight percent of BONTRON E-84®, and a developer was then prepared from this toner in accordance with the procedure of Example IV. The toner exhibited a triboelectric charge of -25.6 microcoulombs per gram, and its rate of charging was measured to be about 10 minutes.

### EXAMPLE VII

A blue toner comprised of 97.0 weight percent of SPAR II® polyester resin, 2.0 weight percent of PV FAST BLUE TM pigment, and 1.0 weight percent of the aluminum complex charge enhancing additive of Example I was prepared by melt blending these three components, followed by micronizing and classifying in accordance with the procedure of Example IV. The resulting toner had a volume average particle diameter of 10.1 microns, and a particle size distribution of 1.31. A developer was prepared from this toner using 2.0 weight percent of toner and a carrier containing a steel core and 0.8 weight percent of a polymer composite coating comprised of 80 weight percent of polymethyl methacrylate and 20 weight percent of VULCAN XC72® carbon black. The toner displayed a triboelectric charge of -10.7 microcoulombs per gram, and its rate of charging was measured to be about 1 minute.

The toner was then surface coated with 0.4 weight percent of AEROSIL R972® by a conventional dry blending method, and a developer was made from this toner and the same carrier particles as before. The triboelectric charge of this toner was measured to be -13.7 microcoulombs per gram, and its rate of charging was 30 seconds.

#### COMPARATIVE EXAMPLE 3

A comparative blue toner and developer composition with a commercial charge additive, BONTRON E-88®, were prepared in accordance with the procedure of Example VII except that BONTRON E-88® was utilized in place of the metal complex charge additive of Example I. The toner displayed a triboelectric charge of -7.5 microcoulombs per gram, and its rate of charging was about 5 minutes.

#### COMPARATIVE EXAMPLE 4

Another comparative blue toner and developer were prepared with the commercial charge additive, BONTRON E-84®, in a similar manner to Comparative Example 3. The triboelectric charge of this toner was -10.5 microcoulombs per gram, and its rate of charging was 15 minutes.

Other modifications of the present invention may occur to those skilled in the art subsequent to a review of the present application, and these modifications, including equivalents thereof, are intended to be included within the scope of the present invention.

What is claimed is:

1. A negatively charged toner composition consisting essentially of resin, pigment or dye particles, optional surface additives, and an aluminum complex composite charge additive containing active charge enhancing components as represented by the following formulas



wherein R is a hydrogen, halogen, alkyl, aryl, alkoxy, aryloxy, hydroxy, nitro, or an amino substituent; Ar represent an aromatic group; M+ is a proton, an alkaline metal cation, or an ammonium ion; and m is a number of from 1 to about 3.

2. A toner composition in accordance with claim 1 wherein M+ is Li<sup>+</sup>, K<sup>+</sup>, Na<sup>+</sup>, Cs<sup>+</sup>, NH<sub>4</sub><sup>+</sup>, R'NH<sub>3</sub><sup>+</sup>, R'₂NH<sub>2</sub><sup>+</sup>, R'₃NH<sup>+</sup>, or R'₄N<sup>+</sup>, wherein the substituents R' of the ammonium ion is an alkyl group containing from 1 to about 10 carbon atoms.

3. A toner composition in accordance with claim 1 wherein the substituents R are tert-butyl groups.

4. A toner composition in accordance with claim 1 wherein the substituents R are halide of iodide, bromide, chloride or fluoride.

5. A toner composition in accordance with claim 1 wherein Ar are the aromatic substituents phenyl, tolyl, xylyl, anisyl, tert-butylphenyl, iodophenyl, diiodophenyl, nitrophenyl, or cyanophenyl.

6. A toner composition in accordance with claim 1 wherein the charge additive is present in an amount of from about 0.1 to about 3 weight percent.

7. A toner composition in accordance with claim 1 wherein the charge additive is incorporated into the toner.

8. A toner composition in accordance with claim 1 wherein the charge additive is present on the surface of the toner composition.

9. A toner composition in accordance with claim 8 wherein the charge additive is contained on colloidal silica particles.

10. A toner composition in accordance with claim 1 wherein the toner's rate of charging is less than about 60 seconds when the toner is frictionally charged against suitable carrier particles via roll milling.

11. A toner composition in accordance with claim 1 with a negative triboelectric charge of from between about -10 to about -40 microcoulombs per gram.

12. A toner composition in accordance with claim 1 wherein the resin is comprised of styrene acrylate, styrene methacrylate, or styrene butadiene.

13. A toner composition in accordance with claim 1 containing a wax component which has a weight average molecular weight of from about 1,000 to about 7,000.

14. A toner composition in accordance with claim 13 wherein the waxy component is selected from the group consisting of polyethylene and polypropylene.

15. A toner composition in accordance with claim 1 wherein the surface additives are metal salts of a fatty acid, colloidal silicas, or mixtures thereof.

16. A toner composition in accordance with claim 1 wherein the pigment is carbon black, magnetites, or mixtures thereof, cyan, magenta, yellow, red, blue, green, brown color pigments or dyes, and mixtures thereof.

17. A toner composition in accordance with claim 1 wherein the charge additive is present in an amount of from about 0.05 to about 5 weight percent.

18. A toner composition in accordance with claim 1 wherein the resin is comprised of styrene polymers, acrylic or methacrylic polymers, polyesters, or mixtures thereof.

19. A toner composition in accordance with claim 1 wherein styrene polymers or polyesters are selected as the toner resin.

20. A developer composition comprised of the toner composition of claim 1 and carrier particles.

21. A developer composition in accordance with claim 20 wherein the carrier particles are comprised of ferrites, steel, or an iron powder with a polymer, or mixtures of polymers, coating thereover.

22. A developer composition in accordance with claim 21 wherein the coating is comprised of a methyl terpolymer, a polyvinylidene fluoride, a polymethyl methacrylate, or a mixture of polymers not in close proximity in the triboelectric series.

23. A developer composition in accordance with claim 20 wherein the carrier particles are comprised of ferrites, steel, or an iron powder with a polymer, or mixtures of polymers, coating thereover.

24. A developer composition in accordance with claim 23 wherein the coating is comprised of a methyl

terpolymer, a polyvinylidene fluoride, a polymethyl methacrylate, or a mixture of polymers not in close proximity in the triboelectric series.

25. A toner in accordance with claim 1 wherein the alkyl or alkoxy group contains from 1 to about 10 carbon atoms; and the aryl group contains from 6 to about 24 carbon atoms.

26. A toner in accordance with claim 25 wherein the alkyl group is methyl.

27. A toner in accordance with claim 1 wherein the aryl group is phenyl, tolyl, xylyl, anisyl, or nitrophenyl.

28. A toner in accordance with claim 1 wherein the active charge enhancing components are selected from the group consisting of potassium (3,5-di-t-butylsalicylato)-bis(4-t-butylphenolato)aluminum (III), (3,5-di-t-butylsalicylato)-bis(phenolato)aluminum (III); (3,5-di-iodosalicylato)-bis(4-t-butyl-phenolato)aluminum (III); (3,5-di-iodosalicylato)-bis(phenolato)aluminum (III); (3,5-di-iodosalicylato)-bis(4-iodophenolato)aluminum (III); (3,5-di-iodosalicylato)-bis(4-iodophenolato)aluminum (III); (3,5-di-iodosalicylato)-bis(3-iodophenolato)aluminum (III); (3,5-di-iodosalicylato)-bis(4-iodophenolato)aluminum (III); (5-iodosalicylato)-bis(3-iodophenolato)aluminum (III); (3,5-di-t-butylsalicylato)-bis(4-methoxy-phenolato)aluminum (III); (3,5-di-iodosalicylato)-bis(3-methoxyphenolato)aluminum (III); (3,5-di-t-butylsalicylato)-bis(4-methylphenolato)aluminum (III); bis(4-t-butylphenolato)-bis(3,5-di-t-butylsalicylato)aluminum (III); bis(phenolato)-bis(3,5-di-t-butylsalicylato)aluminum (III); bis(4-t-butylphenolato)-bis(3,5-di-iodosalicylato)aluminum (III); bis(phenolato)-bis(3,5-di-iodosalicylato)aluminum (III); bis(4-iodophenolato)-bis(3,5-di-iodosalicylato)aluminum (III); bis(3-iodophenolato)-bis(3,5-di-iodosalicylato)aluminum (III); bis(4-iodophenolato)-bis(3,5-di-t-butylsalicylato)aluminum (III); bis(3-iodophenolato)-bis(5-iodosalicylato)aluminum (III); bis(4-methoxyphenolato)-bis(3,5-di-t-butylsalicylato)aluminum (III); bis(3-methoxyphenolato)-bis(3,5-di-iodosalicylato)aluminum (III); and bis(4-methylphenolato)-bis(3,5-di-t-butylsalicylato)aluminum (III).

bis(3,5-di-iodosalicylato)aluminum (III); and bis(4-methylphenolato)-bis(3,5-di-t-butylsalicylato)aluminum (III).

29. A toner in accordance with claim 1 wherein aryl is phenyl, tolyl, xylyl, anisyl, nitrophenyl, or halo-phenyl.

30. A negatively charged toner composition consisting of resin, pigment, and an aluminum complex charge enhancing additive selected from the group consisting of potassium (3,5-di-t-butylsalicylato)-bis(4-t-butylphenolato)aluminum (III), (3,5-di-t-butylsalicylato)-bis(phenolato)aluminum (III); (3,5-di-iodosalicylato)-bis(4-t-butylphenolato)aluminum (III); (3,5-di-iodosalicylato)-bis(phenolato)aluminum (III); (3,5-di-iodosalicylato)-bis(4-iodophenolato)aluminum (III); (3,5-di-iodosalicylato)-bis(3-iodophenolato)aluminum (III); (3,5-di-t-butylsalicylato)-bis(4-iodophenolato)aluminum (III); (5-iodosalicylato)-bis(3-iodophenolato)aluminum (III); (3,5-di-t-butylsalicylato)-bis(4-methoxyphenolato)aluminum (III); (3,5-di-iodosalicylato)-bis(3-methoxyphenolato)aluminum (III); (3,5-di-t-butylsalicylato)-bis(4-methylphenolato)aluminum (III); bis(4-t-butylphenolato)-bis(3,5-di-t-butylsalicylato)aluminum (III), bis(phenolato)-bis(3,5-di-iodosalicylato)aluminum (III); bis(4-t-butylphenolato)-bis(3,5-di-iodosalicylato)aluminum (III); bis(phenolato)-bis(3,5-di-t-butylsalicylato)aluminum (III); bis(4-iodophenolato)-bis(3,5-di-iodosalicylato)aluminum (III); bis(3-iodophenolato)-bis(3,5-di-iodosalicylato)aluminum (III); bis(4-iodophenolato)-bis(3,5-di-t-butylsalicylato)aluminum (III); bis(3-iodophenolato)-bis(5-iodosalicylato)aluminum (III); bis(4-methoxyphenolato)-bis(3,5-di-t-butylsalicylato)aluminum (III); bis(3-methoxyphenolato)-bis(3,5-di-iodosalicylato)aluminum (III); and bis(4-methylphenolato)-bis(3,5-di-t-butylsalicylato)aluminum (III).

\* \* \* \* \*